

Jan. 9, 1951

A. J. MEHLER, JR

2,537,312

HIGH ELONGATION YARN

Filed March 17, 1948

*Fig. 1.*



*Fig. 2.*



INVENTOR.

*Albert J. Mehler, Jr.*

BY

*C. H. Mortenson*

ATTORNEY

## UNITED STATES PATENT OFFICE

2,537,312

## HIGH ELONGATION YARN

Albert J. Mehler, Jr., New Hope, Va., assignor to  
E. I. du Pont de Nemours & Company, Wil-  
mington, Del., a corporation of Delaware

Application March 17, 1948, Serial No. 15,332

3 Claims.

(Cl. 18—54)

1

This invention relates to the manufacture of continuous filament yarns of cellulose acetate having relatively high elongation.

Certain methods for the production of cellulose acetate yarns having relatively high elongation have been described previously. For example, U. S. 2,086,719 describes the production, from solutions of cellulose acetate having viscosities of less than 100 poises at the extrusion temperature, of yarn having dry elongations of about 30% to 40% by stretching the yarn during spinning at a stretch ratio not exceeding 2. While yarns prepared by this method have attractive properties, the required slow rate of spinning at 100 meters per minute or thereabout makes the process unattractive for commercial operation. Attempts to spin at substantially higher spinning speeds, such as several hundred meters per minute or more, while maintaining high elongation yarn properties, have until now been unsuccessful.

Accordingly, it is an object of this invention to furnish filaments and yarns of cellulose acetate having dry elongations about 35% and spun at wind-up speeds in excess of 500 yards per minute. A further object resides in a process for forming continuous filament yarns of cellulose acetate having elongations above 35% and capable of being heat-stretched at relatively low stretch ratio to produce yarns having, after stretching, tensile strengths of 2 grams per denier or more and elongations of 15% to 20%. Other objects will appear hereinafter.

These objects are accomplished by spinning cellulose acetate solutions of relatively high viscosities and preheated to a relatively high temperature into an evaporative atmosphere through relatively small spinneret orifices and under conditions to give a jet velocity of over 600 yards per minute and a stretch ratio of about 0.85 computed on the basis of the spinning wind-up speed divided by the jet velocity of the filament-forming stream issuing from the spinneret assuming no increase or decrease in diameter upon extrusion. For this, the rate of wind-up is greater than 500 yards per minute but is always less than the rate of extrusion. The solution temperature should be at 75° C. to 85° C., being materially higher than the 60° C. head solution temperature normally used.

The present invention will be more easily understood by reference to the following example which is given for illustrative purposes and is not to be considered as limitative.

*Example*

Cellulose acetate prepared from cotton linters and with a degree of polymerization of about 365

2

and a solution viscosity measured at 25% concentration at 40° C. of from 300 to 400 poises was dissolved in acetone to give a solution composed of 25% cellulose acetate, 72.5% acetone and 2.5% water. After deaerating and filtering in the usual manner, the solution was preheated to 80° to 82° C., at which temperature it was extruded through a spinneret having 48 holes, each hole being 0.04 mm. in diameter, into an evaporative spinning cell of the type described in U. S. Patent 1,918,816. The air entering the cell near the spinneret was at 36° C. and became heated to about 90° C. at the point of aspiration near the bottom of the cell at which point it contained about 60 grams of acetone vapor per cubic meter. The rate of spinning solution delivery was maintained at 37 grams per minute equal to a jet velocity of about 700 yards per minute so that the resulting yarn, after separating into two equal parts, measured 75 denier each when wound up at 608 yards per minute. These conditions give a stretch ratio of 0.85 as defined above. A finish was applied to the yarn during wind-up and subsequently the yarn was twisted and wound into a suitable shipping package. The finished yarn had the following properties: 1.28 grams per denier dry tenacity; 37.4% dry elongation; 0.83 grams per denier wet tenacity; and 51.6% wet elongation. The yarn showed a more highly crenulated cross-section than yarns spun heretofore at this high wind-up speed.

It is to be noted that a number of factors have been advantageously combined to produce superior yarn. If the relatively high viscosity solution is spun at normal temperatures of solution extrusion but with all the other factors as above described, yarns of markedly lower elongation result. While it is possible to secure even higher elongations by using a much lower stretch ratio such as of the order of 0.5 or even 0.3, the speed of spinning must be reduced to about 150 yards per minute.

The high elongation yarns of this invention differ from conventional yarns. Figure 1 is a cross-section of a regular 55 denier-18 filament cellulose acetate yarn, and Figure 2 is a cross-section of a 55 denier-18 filament high elongation yarn produced by the process of this invention. From a comparison of the figures, it can be seen that the yarns of this invention are more crenulated than the yarns produced by the normal spinning processes. The greater crenulated nature of the yarns of this invention is desirable because the yarns have greater covering power and fabrics made therefrom are more uniform in appearance.

The high resistance to abrasion and the high

impact strength of the yarns of this invention make them useful where the conventional yarns could not be used satisfactorily. For example, the high elongation yarns of this invention are advantageous in certain specific uses such as in carpet pile yarns and in military cargo chutes. In comparing satins prepared from conventional control yarns and from high elongation yarns of this invention, it was found that the yarns having about 35% greater elongation over the control yarn, gave fabrics which had:

16% higher dry grab strength  
19% higher wet grab strength  
58% higher dry grab elongation  
44% higher wet grab elongation  
66% higher trapezoid tear strength  
7% higher tongue tear strength  
7% higher Mullen bursting strength  
15% higher Taber abrasion resistance

than the fabrics prepared from the control yarn.

Similar results were noted in comparing tricot fabrics prepared from conventional yarn and the high elongation yarns of this invention. The knitted fabrics prepared from yarns of this invention had materially greater fabric strengths (20% or more) than those prepared using conventional yarns.

Fabrics prepared from the high elongation yarns of this invention have dyeing uniformity comparable to controls, more pleasing and softer hand, and, due to the finer denier, can be made sheerer with the same strengths. In addition, the fabrics prepared from the high elongation yarns of this invention did not deluster upon being boiled as much as did conventional fabrics. These advantages may be obtained without sacrifice in mill processing.

It is to be understood, of course, that the above description is for the purpose of illustration only and that my invention is not limited to the exact conditions herein set out but is subject rather to all variations and modifications falling within the terms and spirit thereof as defined in the following claims.

I claim:

1. In a process for spinning cellulose acetate

filaments by extruding a spinning solution of said cellulose acetate, the improvement comprising extruding said solution, containing about 25% of said cellulose acetate and being heated to a temperature of about 80° C. to about 82° C., at a rate of about 700 yards per minute and winding the resultant filaments at a speed of about 608 yards per minute, the ratio of said winding to said extruding being about 0.85.

2. In a process for spinning cellulose acetate filaments by extruding a spinning solution of said cellulose acetate, the steps which comprise extruding said solution at a temperature of about 75° C. to about 85° C. and at a rate exceeding 600 yards per minute jet velocity and winding the resultant filaments at a speed greater than 500 yards per minute but less than said rate of extrusion, the ratio of said winding to said jet velocity being about 0.85.
3. In a process for spinning cellulose acetate filaments by extruding a spinning solution of said cellulose acetate, the steps which comprise extruding said solution at a temperature of about 75° C. to about 85° C. through a spinneret having relatively small holes, said solution having a relatively high viscosity of about 300 to about 400 poises measured at 25% concentration and 40° C. and said extruding being at a rate exceeding 600 yards per minute jet velocity and winding the resultant filaments at a speed greater than 500 yards per minute but less than the rate of extrusion, the ratio of said winding to said jet velocity being about 0.85.

ALBERT J. MEHLER, JR.

#### REFERENCES CITED

The following references are of record in the file of this patent:

#### UNITED STATES PATENTS

| Number    | Name          | Date          |
|-----------|---------------|---------------|
| 2,249,745 | Church et al. | July 22, 1941 |
| 2,290,929 | Whitehead     | July 28, 1942 |
| 2,366,278 | Mehler, Jr.   | Jan. 2, 1945  |
| 2,387,791 | Hoffman       | Oct. 30, 1945 |
| 2,431,435 | Taylor        | Nov. 25, 1947 |